

May 7, 1957

P. S. HESS

2,791,502

FELT PRODUCT AND PROCESS THEREFOR

Filed Dec. 17, 1954



FIG. 1.



FIG. 2.

**INVENTOR**  
PAUL S. HESS.

BY *Joseph C. Harkins Jr.*  
ATTORNEY

2,791,502

**FELT PRODUCT AND PROCESS THEREFOR**

Paul S. Hess, West Orange, N. J., assignor to Cengoleum-Nairn Inc., Kearny, N. J., a corporation of New York

Application December 17, 1954, Serial No. 475,960

12 Claims. (Cl. 92—3)

This invention relates to strengthening agents for cellulosic fibers in felted form and in particular, to new products which are suitable for such use, and to the processes for preparing and incorporating them.

Felted cellulosic fibers impregnated with bituminous materials are frequently employed in the resilient floor and wall covering industry as a backing for linoleum, vinyl, printed felt base and the like. The felt is generally prepared on conventional paper making equipment of the Fourdrinier or cylinder type. It is distinguished from paper in its thickness which ranges from about 0.025 inch to about 0.10 inch and its gauge to weight ratio which ranges from about 1.2 to about 0.8 when measured by the formula

$$\frac{\text{thickness of felt (inches)}}{\text{weight of 480 sq. ft. of felt (pounds)}} \times 1000$$

Various types of felt may be prepared depending on the source of the fibers which are selected and the process of felting them. Some felts employ 100% rags while others may be composed of 100% paper. Any combination of cellulosic fibers may be used, and any given formulation of them as fed to a paper machine is called a "furnish."

For economic and other reasons, it is impossible to prepare a felt as described above which has sufficient strength to function as a backing for floor and wall covering products. It has been the practice therefore to provide additional strength by impregnating the felt with a bituminous material, such as asphalt. Bitumen saturated felt is satisfactory for a great many purposes, but it also has certain disadvantages which the industry has been seeking to overcome. It tends to become brittle when subjected to the high temperatures ordinarily encountered in processing. The color is unpleasing to many consumers. The bitumen tends to migrate from the felt and consequently it is necessary to employ coating materials to prevent possible staining of a wear layer which subsequently may be laminated to the felt. Where very high temperatures are required in processing, as in the case of laminating a vinyl wear layer to a saturated felt backing, problems are encountered with blistering due to the saturant making it difficult to obtain a smooth surface on either side of the final product and more difficult to prevent staining.

While substitutes for the bituminous impregnants have long been sought, only a few have reached the stage of being employed commercially. One such substitute comprises a mixture of tall oil, a plasticizer therefor, and an organic solvent. This mixture has proved objectionable for widespread use because it gives rise to a great hazard of fire and explosion. The problem of solvent evaporation contributes to this danger, but more importantly, there is a likelihood of spontaneous combustion due to the oxidation of the unsaturated aliphatic acids which are present. The mere "drying" and/or "gelling" of the mixture after it has been incorporated in felt at the required temperatures of from about 180° F. to about 200° F.

has resulted in numerous fires. The "stoving" of linoleum which is backed with such felt must be carefully controlled, and serious fires and explosions have occurred in spite of the closest observation.

5 The present invention provides a greatly improved impregnant for floor and wall covering felt. It overcomes many of the disadvantages of bituminous impregnants and permits the safe use of a tall oil compound.

Because it has been impossible to ascertain the precise 10 chemical composition of the product of the present invention, it is described hereafter in terms of the preferred process of preparing it. Briefly stated, an ester of a polyhydric alcohol and tall oil is oxidatively polymerized by heating it in the presence of excess oxygen until it has achieved a viscosity of from about 2,000 centipoises to about 10,000 centipoises, and thereafter it is further heated in the absence of oxygen and at a higher temperature until it reaches a viscosity of at least about 30,000 centipoises, although it is not permitted to reach a condition 15 whereafter gelling cannot be prevented. The oxidized and polymerized tall oil ester is then cooled to minimize further polymerization. A water emulsion of the above product may be prepared and the emulsion used as an impregnant for felt in accordance with well-known techniques. It is usually desirable to "cure" or gel the impregnant after it has been incorporated in the felt by subjecting it to elevated temperatures.

The product of the invention when used as a felt impregnant eliminates the problems of staining and makes 20 unnecessary the use of expensive seal coats. It provides a more attractive product in that it has a light color, and it does not smear off when it brushes against furniture or the like during handling and installation as does asphalt. It does not blister at high temperatures and 25 therefore provides a smoother product when a vinyl wear layer is laminated to it. In this regard, there is considerably less loss of goods in processing because when a vinyl product prepared in the usual way contains too many and/or too large blisters, it is treated as waste.

30 A principal advantage of the product of the invention is its resistance to oxidation. It is believed that the first step of the process; namely, the oxidation of the tall oil ester to a condition measured by a viscosity of between about 2,000 and 10,000 centipoises, effects oxidative polymerization of the ester by forming peroxides at 35 the oxygen containing functional groups which in turn react with similar peroxide groups to form oxygen linkages. The second step of the process apparently effects further polymerization by the creation of linkages between carbon atoms; it also destroys any unreacted peroxide groups. If the second stage of polymerization is not permitted to reach a stage whereafter it is impossible to prevent gelling but does reach a degree of polymerization indicated by a viscosity of at least about 30,000 centipoises, the product of the invention is obtained which 40 upon cooling is water emulsifiable and contains a number of oxygen reactive groups small enough to eliminate any fire or explosion hazard. On the other hand, the product is strong enough for use as a felt impregnant. While the invention is not predicated on the above theory, it is 45 helpful by way of explanation in regard to the control of the process.

The first stage of oxidative polymerization is best conducted at a temperature of below about 260° F. and 50 preferably at about 210° F. At higher temperature, peroxide groups are destroyed too rapidly, thereby decreasing the number of oxygen linkages formed to a point below that necessary for achieving the product of the invention. Excess oxygen must be supplied at the first 55 stage to permit the rapid formation of the peroxide groups. It may be supplied in any conventional manner; for example, by bubbling it through the reaction vessel.

Generally, the ester requires from about 4 to about 6 hours to reach the desired viscosity, exclusive of the time required for it to reach the reaction temperature.

The second stage of polymerization may follow the first stage immediately, and this is preferred, or it may follow it by a considerable period of time if the product of the first stage is kept at a low temperature on the order of below about 70° F. The difficulty with the latter procedure is that reaction, once started, continues to some extent at any temperature, and after a period of time the second stage of polymerization cannot adequately be controlled. In either event, however, the second stage is conducted in the absence of oxygen and preferably at a temperature of from about 520° F. to about 590° F. although any temperature is satisfactory if the aforementioned viscosity condition can be reached without gelation. At lower temperatures, the rate of carbon to carbon linking is slow and unreacted peroxide groups may not be destroyed. At higher temperature polymerization is too rapid to be satisfactorily controlled to prevent eventual gelling. It is preferable to pass carbon dioxide through the reaction vessel during the second stage to remove any water which is formed. It is also the best practice to cool the product when it has reached the desired viscosity during the second stage to prevent further reaction.

It has been found that the minimum viscosity of 30,000 centipoises required after the second stage of polymerization is important in providing a product which has the strength needed for use in floor and wall covering felt. Any degree of polymerization represented by a higher viscosity may be used provided a substantial amount of gelling is not encountered prior to emulsification, but it becomes increasingly difficult to control the process in regard to gelling as the higher viscosities are sought. As the viscosity increases, the size of the combining molecules increases and each subsequent linking effects a greatly increased viscosity. In addition, subsequent emulsification becomes more difficult. For these reasons, it is preferred to maintain a viscosity in the second stage of polymerization below about 150,000 centipoises.

Emulsification of the product of the second stage of polymerization is easily accomplished, and it is preferred to employ an emulsifying agent such as morpholine, other amines, or the like. The emulsion may then be applied to felt by means of a coating apparatus or by dipping in a conventional manner, although it is usually desirable that the felt be supported during such an operation as it has a very low wet strength. Once the emulsion is incorporated in felt, it must be cured or gelled to provide the strength needed for floor and wall covering products. The rate of gelling is accelerated by elevated temperatures and consequently their use is preferred. The proper degree of gelling must be determined empirically and therefore no standard conditions of time and temperature can be set forth. Curing conditions of 250° F. for six hours followed by 180° F. for 21 days and 325° F. for 2 hours followed by 180° F. for 21 days have proved satisfactory. If a wear layer that requires stoving is to be laminated to the impregnated felt, all or a portion of the cure may be effected during stoving. Linoleum is generally stoved at temperatures of about 180° F. to 200° F. for from 10 to 30 days, and printed felt base is generally stoved for 2 to 5 days at the same temperatures. Preliminary curing prior to stoving or other treatment for from 30 minutes to 6 hours at temperatures ranging from about 180° F. to 325° F. is usually desirable in order to provide sufficient strength in the impregnated felt for handling and processing it. Where no stoving is intended, curing may be conducted at higher temperatures and the time required therefor is considerably decreased. Gelling apparently is a continuation of polymerization, which, if conducted in the presence of a sufficient number of oxygen reactive groups, would give rise to the aforementioned fire and explosion hazard.

By conducting the second stage of the process in the absence of oxygen is meant simply that large amounts of oxygen are not permitted to be dispersed throughout the tall oil ester at this point. The reaction may be conducted in an ordinary reaction vessel which is exposed to the atmosphere, and the reactants may be agitated or stirred in the course of polymerization. A single reaction vessel may conveniently be employed for both stages of the process.

When using the product of the invention as a replacement for an asphalt impregnant, it has been found that about half as much of the modified tall oil ester based on the bone dry weight of the felt is required to achieve comparable strength, flexibility and stiffness values. For example, a product containing 120 parts of asphalt per 100 parts of felt has a tensile strength after 21 days of stoving, as measured by the Scott test, of 175. The Mullen bursting strength is 220 and the tear strength measured by the Thwing-Albert machine is 5.8. The flexibility as measured by the Mandrel test is one-half inches and the stiffness measured by the Suvant apparatus is 350. A product which is identical, except that 60 parts of the modified tall oil ester of the invention per 100 parts of bone dry felt is employed instead of the asphalt, has a Scott of 173; a Mullen of 225; a Thwing-Albert reading of 4.8; a Mandrel reading of one-half inch; and a Suvant of 225. The above tests are well known, being used by a number of manufacturers of impregnated felt products to ascertain the indicated characteristics.

It is generally undesirable to use more than about 75% of the modified tall oil ester of the invention in relation to the amount of bituminous material that ordinarily would be used to obtain given properties. If excessive amounts are used, the felt becomes extremely stiff over relatively short periods of time, and since the rate of stiffening is accelerated by elevated temperatures, stoving accentuates the problem. For the usual type of floor and wall covering felts, the aforementioned amount of about 50% is most preferred although amounts as low as 25% provide felts suitable for speical needs.

Many tall oil esters of polyhydric alcohols are suitable as starting products in the present invention. Tall oil is obtained as a by-product in the manufacture of sulfate pulp from pine trees, and it contains varying amounts of rosin acids, drying oil fatty acids and unsaponifiable matter depending on its source and the degree of refining it has undergone. American refined tall oil is generally preferred in the practice of the invention. Esterification of tall oil with a polyhydric alcohol is a well-known reaction; however, the ester referred to herein is that of the polyhydric alcohol and the fatty acids present in tall oil, there being no, or little, esterification of the rosin acids. This product is sometimes called a half ester.

The polyhydric alcohol employed in the esterification must contain at least three reactive hydroxy groups. If it contains less, the ester cannot be modified as described herein to provide sufficient strength for use in floor and wall covering felt. Pentaerythritol, which contains four reactive hydroxyl groups, is most preferred. Although glycerol esters have proved satisfactory for certain uses, they have less strength when used as an impregnant than do the most preferred pentaerythritol esters. Moreover, the glycerol esters require more time in processing, particularly during the second stage of polymerization, and take a longer time to completely gel after impregnation. The modification of tall oil esters of polyhydric alcohols having more than four hydroxyl groups results in stiffer final products and are more difficult to control in preparation. Where stiffness is not a serious problem, as in a backing material for tile, a tall oil ester of sorbitol may be used.

A process for preparing the product of the invention is set forth at Fig. 1 of the drawings and a detailed example of a preferred embodiment of the invention is de-

scribed hereafter in connection therewith. The tall oil used in preparing the ester is American refined tall oil containing 68% fatty acids of which 36.5% is linolenic acid, 19% is linoleic acid and 43.7% is oleic acid; 30% rosin acids; and 2% unsaponifiable matter. The tall oil is reacted with a stoichiometric amount of technical pentaerythritol with reference to the amount of fatty acids which are present, and the ester or half ester is thereafter separated. In the present example, 1000 pounds of the ester are introduced to the reaction vessel 1 which is heated by means of a steam jacket (not shown) to a temperature of 212° F. About 30 minutes are required for the ester to reach the desired temperature. Oxygen is passed through the reaction vessel from the time the ester is introduced. The amount of oxygen is sufficient provided it is being evolved from the reaction vessel. The reaction is allowed to continue for 4 hours at 212° F. at which time it has a viscosity of 5,000 centipoises as measured by a Brookfield Viscometer. The ester is then passed to reaction vessel 2 which is heated by a steam jacket (not shown) to 570° F. and CO<sub>2</sub> is continuously passed through the contents of the vessel. After 2 hours the ester reaches a temperature of 570° F. and after 30 minutes a viscosity of 30,000 centipoises as measured by a Brookfield Viscometer. The ester is then quickly passed to a cooling chamber 3 where it is reduced in temperature to below 212° F. It is emulsified at 4 by adding 4 parts of morpholine and 100 parts of water for each 100 parts of modified tall oil ester. It is then stored at 5 until needed. The container 5 may be at room temperature.

When the modified ester is to be used as an impregnant for felt, as shown in Fig. 2, it is removed from storage at 5 and passed to a dip tank 8 at a rate sufficient to keep the tank adequately supplied. A previously prepared 100% cotton rag felt containing about 4% moisture is fed from a roller at 6 to a conveyor 7 where by means of roller 9 it is immersed in dip tank 8. The felt remains in the dip tank for 0.05 second after which it has a moisture content of 50% based on the bone dry weight of the felt. Thereafter it is passed through an air heated chamber 10 where the moisture is substantially completely removed. The impregnated felt is then heated at 200° F. for 3 hours. It has a final modified tall oil pentaerythritol ester content of 60% and the aforesaid strength, flexibility and stiffness characteristics as well as the other desirable properties herein discussed. At no point in the process is there a fire or explosion hazard and the same do not exist with regard to any subsequent use which is made of the product.

While the above invention has been described in connection with specific and detailed examples, it is not to be limited thereby. Modifications and variations intended to be within the scope of the invention will be apparent to those skilled in the art and therefore reference is to be had to the appended claims for the limits of the scope of the invention.

What is claimed is:

1. A process for modifying an ester of tall oil, said ester containing free rosin acids in substantially the amount supplied by the tall oil, the fatty acid content of said ester being substantially completely esterified with a polyhydric alcohol having at least three hydroxyl groups, which comprises the steps of: first, heating the ester at a temperature of less than 260° F. in the presence of excess oxygen until it has a viscosity of from about 2,000 to about 10,000 centipoises; second, heating the product of the first step in the absence of oxygen until it has a viscosity of at least about 30,000 centipoises, said viscosity also being less than that at which gelling of the ester will occur; and third, cooling the product of the second step to a temperature of less than about 210° F.

2. A process for modifying an ester of tall oil, said ester containing free rosin acid in substantially the amount supplied by the tall oil, the fatty acid content of said

ester being substantially completely esterified with a polyhydric alcohol having at least three hydroxyl groups, which comprises the steps of: first, heating the ester at a temperature less than about 260° F. in the presence of excess oxygen until it has a viscosity of from about 2,000 to about 10,000 centipoises; second, heating the product of the first step at a temperature within the range of from about 520° F. to about 590° F. in the absence of oxygen until it has a viscosity of at least about 30,000 centipoises, said viscosity also being less than that at which gelling of the ester will occur; and third, cooling the product of the second step to a temperature of less than about 210° F.

3. A process according to claim 2 wherein the polyhydric alcohol is pentaerythritol.

4. A process for modifying an ester of tall oil, said ester containing free rosin acids in substantially the amount supplied by the tall oil, the fatty acid content of said ester being substantially completely esterified with a polyhydric alcohol having at least three hydroxyl groups, which comprises the steps of: first, heating the ester at a temperature of less than 260° F. in the presence of excess oxygen until it has a viscosity of from about 2,000 to about 10,000 centipoises; second, heating the product of the first step in the absence of oxygen until it has a viscosity of at least about 30,000 centipoises and less than 150,000 centipoises, said viscosity also being less than that at which gelling of the ester will occur; and third, cooling the product of the second step to a temperature of less than about 210° F.

5. The process of claim 4 wherein the heating in the presence of excess oxygen is carried out for a period of about four to six hours.

6. The process of claim 5 wherein the polyhydric alcohol is pentaerythritol.

7. A liquid composition suitable for impregnating felt and which can be converted to a solid material by the application of heat which comprises an ester of tall oil having a viscosity of from about 30,000 to about 150,000 centipoises, said ester containing free rosin acid in substantially the amount supplied by the tall oil and the fatty acid content of said ester being substantially completely esterified with a polyhydric alcohol having at least three hydroxyl groups, said ester having been preliminarily heated at a temperature of less than 260° F. in the presence of oxygen until it had a viscosity of from about 2,000 to about 10,000 centipoises and thereafter heated in the absence of oxygen to increase its viscosity.

8. An emulsion suitable for impregnating felt which is converted to a solid residue by the application of heat which comprises water and dispersed therein an ester of tall oil having a viscosity of from about 30,000 to about 150,000 centipoises, said ester containing free rosin acid in substantially the amount supplied by the tall oil and the fatty acid content of said ester being substantially completely esterified with a polyhydric alcohol having at least three hydroxyl groups, said ester having been preliminarily heated at a temperature of less than 260° F. in the presence of oxygen until it had a viscosity of from about 2,000 to about 10,000 centipoises and thereafter heated in the absence of oxygen to increase its viscosity.

9. An emulsion suitable for impregnating felt which is converted to a solid residue by the application of heat which comprises water and dispersed therein an ester of tall oil having a viscosity of from about 30,000 to about 150,000 centipoises, said ester containing free rosin acid in substantially the amount supplied by the tall oil and the fatty acid content of said ester being substantially completely esterified with pentaerythritol, said ester having been preliminarily heated at a temperature of less than 260° F. in the presence of oxygen until it had a viscosity of from about 2,000 to about 10,000 centipoises and thereafter heated in the absence of oxygen to increase its viscosity.

10. A sheet of felted cellulosic fibers having when dry a thickness of at least about 0.025 inch and less than about 0.10 inch and a gauge to weight ratio of from about 0.8 to about 1.2 when measured by the formula

$$\frac{\text{felt thickness (inches)}}{\text{weight of 480 square feet of felt (pounds)}} \times 1000$$

having dispersed throughout said sheet a liquid ester of tall oil which is converted to a solid material by the application of heat, said ester having a viscosity of from about 30,000 to about 150,000 centipoises and containing free rosin acid in substantially the amount supplied by the tall oil and the fatty acid content of said ester being substantially completely esterified with a polyhydric alcohol having at least three hydroxyl groups, said ester having been preliminarily heated at a temperature of less than 260° F. in the presence of oxygen until it had a viscosity of from about 2,000 to about 10,000 centipoises and thereafter heated in the absence of oxygen to increase its viscosity.

11. A process for preparing a sheet of felted cellulosic fibers impregnated with a strengthening agent which comprises depositing a slurry of loose cellulose fibers on a base in the form of a sheet and removing the moisture therefrom to provide a dry sheet having a thickness of at least about 0.025 inch and less than about 0.10 inch and a gauge to weight ratio of from about 0.8 to about 1.2 when measured by the formula

$$\frac{\text{felt thickness (inches)}}{\text{weight of 480 square feet of felt (pounds)}} \times 1000$$

applying a water emulsion of a modified tall oil ester to said dry sheet of felted fibers, drying the sheet to remove the water and gelling the modified ester in the sheet at an elevated temperature, said modified tall oil ester being prepared from a tall oil ester containing free rosin acids in substantially the amount supplied by the tall oil, the fatty acid content thereof being substantially completely esterified with a polyhydric alcohol having at least three hydroxyl groups, and said tall oil ester being modified by first, heating the ester at a temperature of less than 260° F. in the presence of excess oxygen until it has a viscosity of from about 2,000 to about 10,000 centipoises; second, heating the product of the first step in the absence of oxygen until it has a viscosity of at least about 30,000 centipoises, said viscosity also being less than that at which gelling of the ester will occur; and third,

cooling the product of the second step to a temperature of less than about 210° F.

12. A process for preparing a sheet of felted cellulosic fibers impregnated with a strengthening agent which comprises depositing a slurry of loose cellulose fibers on a base in the form of a sheet and removing the moisture therefrom to provide a dry sheet having a thickness of at least about 0.025 inch and less than about 0.10 inch and a gauge to weight ratio of from about 0.8 to about 1.2 when measured by the formula

$$\frac{\text{felt thickness (inches)}}{\text{weight of 480 square feet of felt (pounds)}} \times 1000$$

dipping said dry sheet of the felted fibers in a water emulsion of a modified tall oil ester, removing substantially all of the free moisture from the sheet and partially gelling the modified ester in the sheet by heating it at a temperature within the range of from about 180° F. to about 375° F. for from about 30 minutes to about 360 minutes, said modified tall oil ester being prepared from a tall oil ester containing free rosin acids in substantially the amount supplied by the tall oil, the fatty acid content thereof being substantially completely esterified with pentaerythritol and said tall oil ester being modified by first, heating the ester at a temperature of about 210° F. in the presence of excess oxygen until it has a viscosity of from about 2,000 to about 10,000 centipoises; second, heating the product of the first step at a temperature of about 570° F. in the absence of oxygen until it has a viscosity within the range of from about 30,000 centipoises to about 150,000 centipoises, said viscosity also being less than that at which gelling of the ester will occur; and third, cooling the product of the second step to a temperature of less than about 210° F.

35 References Cited in the file of this patent

UNITED STATES PATENTS

|           |             |       |               |
|-----------|-------------|-------|---------------|
| 2,041,836 | Hunt        | ----- | May 26, 1936  |
| 2,317,487 | Schuelke    | ----- | Apr. 27, 1943 |
| 2,346,934 | Miller      | ----- | Apr. 18, 1944 |
| 2,365,300 | Segesemann  | ----- | Dec. 19, 1944 |
| 2,382,297 | Cupery      | ----- | Aug. 14, 1945 |
| 2,424,074 | Bent et al. | ----- | July 15, 1947 |
| 2,435,831 | Harvey      | ----- | Feb. 10, 1948 |
| 2,447,506 | Jubanowsky  | ----- | Aug. 24, 1948 |
| 2,493,486 | Greenlee    | ----- | Jan. 3, 1950  |
| 2,494,559 | Jubanowsky  | ----- | Jan. 17, 1950 |
| 2,516,104 | Burrell     | ----- | July 25, 1950 |